

## UNITED STATES PATENT OFFICE

2,121,949

BITUMINOUS PAINT AND METHOD OF  
MAKING THE SAME

Edward James Canavan, Teaneck, N. J., assignor  
to The Barrett Company, New York, N. Y., a  
corporation of New Jersey

No Drawing. Application February 7, 1934,  
Serial No. 710,110

2 Claims. (Cl. 134—51)

This invention relates to bituminous paints, and more particularly, to bituminous paints or coating compositions for protecting metal surfaces having oil or grease spots, i. e., films of oil or grease, thereon and to procedures for making such paints and protecting such surfaces.

Metal pipes, and particularly steel pipes, which are coated in the field with coal tar pitch are usually primed at the mill with a coal tar paint or primer. The priming coat must be continuous, i. e., free of bare spots. Otherwise, while in transit, rust spots will develop on the pipes. The bare spots in the priming coat may be largely due to oil or grease adhering to the pipe walls and preventing adhesion of the priming coat to the metal surface of the pipe. In practice, it has been found expensive and practically impossible to completely remove the oil or grease from the pipe surface at the mill where the pipe is formed and to maintain the surface entirely free from films of oil or grease until the pipe is primed or painted. Consequently, as heretofore practiced, the priming of the pipe at the mill with coal tar primers has resulted frequently in poorly primed pipes. This may be attributed to the fact that bituminous paints, and particularly tar pitch paints, such as coal tar pitch and water gas tar pitch, when applied to steel or other metal surfaces contaminated with lubricating oil or grease, which are generally not miscible with the paint, fail to form a continuous coating over the metal surface. Hence, bare spots are left on the metal which permit subsequent corrosion of the metal when it is exposed to weathering influences. For example, in the manufacture of electrically welded steel pipes for gas lines, the pipe surface often contains spots and streaks of lubricating oil picked up by the pipe in its passage through the forming rolls and conveying equipment of the electric welding apparatus. Such oily spots or streaks may be hardly perceptible in a casual examination but yet be sufficient to cause a faulty coating when the bituminous paint is applied.

It is an object of this invention to provide a bituminous paint, and more particularly, a tar-pitch paint, which, when applied to steel or other metal surfaces bearing lubricating oil or grease, will form a continuous coating completely covering the metal surface and thus efficiently protect it against corrosion. Other objects and advantages will appear from the following detailed description.

I have found that even if an oil or grease film or spot be present on the metal pipe, it can be properly primed with a bituminous paint such as

a tar pitch paint having incorporated therein a soap or other material having detergent properties in the presence of organic solvents. The addition of a metallic salt of a fatty acid, e. g., a soap, to a bituminous paint or coating composition, I have found modifies the same so that it wets and flows evenly over lightly oiled metal surfaces, resulting in the formation of a continuous paint film or coating on such surfaces. Aluminum stearate is preferred for use in this invention because of the highly satisfactory results obtained in priming oil-spotted metal pipes, such as steel pipes, with the coal tar paint in which this material was incorporated, as herein-after more fully described. The addition of aluminum stearate to pitch paints, and particularly to coal tar pitch or water gas tar pitch paints, modifies the surface tension and wetting characteristics of the paint so that it readily coats metal surfaces, including any oil or grease-bearing portions thereof, forming a continuous paint film which effectively protects the metal. Among the detergent materials which may advantageously be used in pitch paints are: other metallic salts of fatty acids such as magnesium stearate, zinc stearate, zinc laurate, ammonium and substituted ammonium soaps soluble in organic solvents, and salts of certain sulphonic acids having detergent properties in the presence of organic solvents, e. g., sodium salts of naphthalene sulphonic acids.

One example of a tar-pitch paint produced in accordance with my invention is given below:

A pitch base, consisting essentially of coal tar pitch, and having a melting point of from 143° F. to 148° F. and a maximum percentage of "free carbon" of approximately 12 per cent, was melted. Crude solvent naphtha was then added to the melted pitch in such quantity that the resultant mixture had an Engler viscosity for 100 c. c. at 25° C. of from 175 to 225 seconds.

The aluminum stearate solution was prepared by adding approximately seven ounces of aluminum stearate to one gallon of crude solvent naphtha, thus forming a solution containing approximately 5 per cent by weight of aluminum stearate. The mixture was heated slowly to a temperature of from 70° to 80° C., at which temperature a gel was formed. The temperature was then slowly raised to 170° C. and the mixture held at that temperature for about ten minutes. During the second stage of heating, the gel-like mass changed to a syrupy solution which when cooled to about 30° C. exhibited frothing properties. The paint was made by mixing 80 parts

of the pitch : solvent naphtha mixture with 20 parts of the aluminum stearate : solvent solution. The finished paint contained approximately 1 per cent of aluminum stearate by weight; i. e., about 1.4 ounces of stearate per gallon of paint.

An important feature of this invention is the procedure following in incorporating the metallic soap in the paint. I have found that the heating of the aluminum stearate or other soap employed admixed with the solvent to a sufficiently high temperature (in the example above given, 170° C.), the gel originally formed becomes fluid and changes to a syrup which remains a syrup on cooling. The cooled syrup can readily be mixed with the other paint ingredients.

The pitch base employed in the paint may be coal tar pitch, water gas tar pitch, coal tar, water gas tar, mixtures of these pitches or tars, or other bituminous materials. The amount of pitch used in the paint may vary from 40 to 65 per cent by volume of pitch while the amount of solvent employed may vary from 35 to 60 per cent. However, when a paint of slow drying characteristics is desired, the percentage of soft pitch may be as high as 80 per cent, the proportion of solvent being reduced correspondingly. When the base of the paint consists of tar or soft distilled tars, the percentage of solvent may be reduced below 20 per cent, but ordinarily 10 per cent or more of solvent is necessary in a paint of suitable drying properties and hardness of paint coating.

In lieu of employing a solution of aluminum stearate or other metallic soap containing approximately 5 per cent by weight of metallic soap, as in the example above given, an aluminum stearate solution or other metallic soap solution containing up to approximately 20 per cent by weight of metallic soap may be employed. The 5 per cent solution, it was found, did not substantially alter the viscosity of the paint when added thereto. As the addition of a 20 per cent solution of aluminum stearate to the pitch : solvent mixture would alter the viscosity, a mixture of pitch and solvent of lower viscosity may be used with the 20 per cent solution than is used with a 5 per cent solution, so that the finished paint has substantially the same viscosity as the paint of the example hereinabove given. If a low viscosity paint is desired, aluminum stearate solu-

tions containing less than 5 per cent of aluminum stearate by weight may be employed, or a mixture of pitch and solvent of lower viscosity may be combined with a solution of metallic soap containing at least 5 per cent of metallic soap. The amount of aluminum stearate in the finished paint may vary from 0.5 per cent to 5 per cent by weight, 1 per cent by weight of aluminum stearate being preferred.

Instead of the solvent naphtha, drip oil, coke oven light oil, or distillates obtained from coal tar, water gas tar, or the oils mentioned may be employed to flux the coal tar pitch, water gas tar pitch, coal tar or other bituminous base employed in making the paint. Preferably, the boiling point of the solvent or flux used should be within the range of from 100° C. to 220° C. Other organic liquids may be employed as solvents for the pitch in the manufacture of the paint, as for example carbon tetrachloride.

The paint may be applied to the metal or other surface either by spray or brush application or by dipping the metal surface into a bath of the paint.

It is to be understood that this invention is not restricted to the present disclosure otherwise than defined by the appended claims.

I claim:

1. A fluid, brushable paint consisting of from 40 to 65 percent by volume of pitch from the group consisting of coal tar pitch and water gas tar pitch, from 35 to 60 percent by volume of solvent for said base, and a small amount of aluminum stearate dissolved in said solvent whereby said aluminum stearate is permanently and homogeneously distributed in dissolved form through said paint.

2. The process of making a bituminous paint containing from .5 per cent to 5 percent by weight of aluminum stearate which comprises mixing said aluminum stearate with solvent naphtha, heating the resultant mixture to a temperature of from 70° to 80° C. until a gel is formed, continuing the heating until the gel is changed to a syrup, cooling the syrup and mixing the same with a mixture comprising pitch derived from coal and 10 to 60 per cent by volume of a solvent therefor.

EDWARD JAMES CANAVAN.